

Feb. 11, 1930.

S. DUSHMAN

1,747,061

ELECTRODE COMPOSITION FOR ELECTRON DISCHARGE DEVICES

Filed July 2, 1923



Inventor:  
Saul Dushman,  
by *Alexander S. Flint.*  
His Attorney.

## UNITED STATES PATENT OFFICE

SAUL DUSHMAN, OF SCHENECTADY, NEW YORK, ASSIGNOR TO GENERAL ELECTRIC COMPANY, A CORPORATION OF NEW YORK

## ELECTRODE COMPOSITION FOR ELECTRON-DISCHARGE DEVICES

Application filed July 2, 1923. Serial No. 648,875.

The present invention relates to the constitution of cathodes for electrical discharge devices, as for example, radio detectors, rectifiers and the like.

5 The object of my invention is to provide a cathode material capable of high electron emission at an operating temperature which is relatively low and which therefore permits of operation of the device by a low heating current capable of being furnished by an ordinary primary battery.

10 I have found that the element yttrium is capable of a commercially useful electron emission at a temperature as low as about 1300 degrees C. In accordance with my invention an oxide of yttrium is incorporated into an electrode which is operated under conditions permitting reduction of at least 15 part of the yttrium, whereby the electron emissivity of the electrode is very materially improved.

20 When making an electrode embodying my invention, a finely divided yttrium compound is incorporated with the material constituting the main body of the electrode, as 25 distinguished from a surface application. For example, in the manufacture of a tungsten cathode embodying my invention, a suitable non-volatile compound of yttrium is 30 mixed with the finely divided metallic tungsten from which cathode filaments are fashioned either in accordance with the Coolidge mechanical working process described in the United States Patent No. 1,082,933 of 35 December 30, 1913, or by squirting of the 40 finely divided material admixed with a suitable binder.

When manufacturing drawn tungsten cathodes about one to two per cent of an oxide of yttrium  $Yt_2O_3$  or  $YtO_2$ , or other suitable non-volatile compound of yttrium is 45 mixed with the finely divided tungsten metal before it is pressed into slugs preparatory to sintering. In general, as much yttrium compound is added as may be tolerated in the

tungsten without interfering with the subsequent swaging and drawing in accordance with Coolidge Patent No. 1,082,933.

In some cases it may be more convenient to form electrode from a mixture of metal and an yttrium compound by adding a suitable binder in sufficient quantity to produce a plastic mass and squirting the same into filaments or ribbons. For example, filaments may be made by squirting a mixture comprising by weight about 95 parts tungsten, 50 about 5 parts yttria,  $Yt_2O_3$  and enough carbonaceous binder to form a mass capable of being squirted, and thereafter baking, treating to remove the binder, and sintering in the 55 usual way.

When filaments made in this way are mounted as cathodes in an electron discharge device, for example, such as shown in the drawing, comprising a bulb 1, a cathode 2, an anode 3 and a grid 4, precautions should be taken to thoroughly evacuate the bulb and contained parts, especially to remove water vapor. The electron device is provided as usual with the cathode leads 5, 6 and anode lead 7 and a grid lead 8, all of which are sealed into a stem 9 and connected to terminals (one numbered 10 being shown) sealed into a base 11. However, as these structural features form no essential part of my invention they will not be described in greater detail. Preferably, but not necessarily a material of low vapor pressure which is highly reactive to water vapor, as for example, magnesium or calcium, is introduced into the 70 bulb. In the device shown in the drawing, this material for removing traces of water vapor is indicated as a film 12 on the bulb wall.

When the evacuation is complete and preferably when the bulb has been sealed, the cathode is activated by heating to a temperature of about 2300 degrees C. for about a minute, and then formed at about 1300 degrees to 1450 degrees C. for a few minutes. 85 90

Heating to 2300 degrees C. results in a reduction of a small part of the yttria to yttrium, which diffuses at the forming temperature to the cathode surface where it remains in greater part as an adsorbed film. The temperature of normal operation preferably is materially lower, usually below 1300 degrees C. as at the higher temperatures yttrium tends to be vaporized from the incandescent

10 tungsten. At 1450 degrees C. the evaporation is quite rapid. In general, cathodes containing yttrium as a constituent should be operated at a red heat below incandescence. Cathodes containing yttria after having been 15 activated and formed as above described, when operated at about 1300 degrees C. give an electron emission of at least about 10 milliamperes per sq. cm. of emitting surface, whereas pure tungsten at the same temperature has the extremely low electron emission 20 of about 0.0008 of a milliampere per sq. cm.

Conveniently, but not necessarily, a non-volatile reducing agent, such as carbon, is incorporated with the yttria into the cathode in 25 order to assist in reducing the yttria particularly when for any reason water vapor is evolved even though in minute quantity during the operation of the device. Carbon may be introduced by heating the filament in the 30 presence of the vapor of a carbon compound, as for example, the vapor of anthracene or naphthalene. The pressure of this vapor should be maintained at a low value and the temperature of the cathode, the time of treatment 35 and other conditions should be so regulated as to maintain the carbon content less than about one per cent and preferably as low as about one-half per cent.

Although the manufacture of a tungsten 40 base electrode has been described for the purpose of illustrating my invention, I wish it to be understood that the benefits of my invention also may be obtained in the case of electrodes consisting wholly or largely of other 45 metals, as for example, molybdenum or nickel.

What I claim as new and desire to secure by Letters Patent of the United States, is:

1. The process of treating an electrode containing yttrium as a constituent which consists in heating said electrode in non-oxidizing 50 environment to about 2300 degrees C. then heating to about 1300 to 1450 degrees C. and finally operating said electrode at a lower temperature.

55 2. The process of treating an electrode containing yttrium as an elementary constituent in a non-oxidizing environment which consists in heating said electrode to about 2300 degrees C. for about one minute, then heating to about 1300 to 1450 degrees C. for several minutes, and finally operating said electrode at a temperature of about 1300 degrees C.

60 3. The process of treating a tungsten electrode containing an oxide of yttrium for use

in an electron discharge device which consists in heating said electrode to about 2300 degrees C. for about one minute, then heating to about 1300 degrees to 1450 degrees C. for several minutes, and finally operating said electrode at a temperature of about 1300 degrees C., all of said operations being carried out in a vacuum free from traces of water vapor.

In witness whereof, I have hereunto set my hand this 30th day of June, 1923.

SAUL DUSHMAN.

8

8

9

9

10

10

11

11

12

12

13